

July 25, 1939.

C. F. R. HARRISON ET AL

2,167,112

PREPARATION OF NICKEL CARBONYL

Filed Nov. 8, 1934



Charles Frederick Reed <sup>INVENTORS</sup>  
Harrison  
and Albert Edward Wallis  
BY

Byers, Stilhuis & Blodoo  
ATTORNEYS

## UNITED STATES PATENT OFFICE

2,167,112

## PREPARATION OF NICKEL CARBONYL

Charles Frederick Reed Harrison, Selley Oak, Birmingham, and Albert Edward Wallis, Clydach, England, assignors to The International Nickel Company, Inc., New York, N. Y., a corporation of Delaware

Application November 8, 1934, Serial No. 752,076  
In Great Britain November 11, 1933

5 Claims. (Cl. 23—203)

This invention relates to the separation of nickel carbonyl in the liquid phase from a mixture of gases and vapours containing it. Nickel carbonyl is usually made by treating reduced nickel with carbon monoxide at atmospheric pressure, and it may be made by treating reduced nickel, or nickel matte or other impure source of nickel with carbon monoxide at high pressure. The resultant gases contain nickel carbonyl together with substantial quantities of carbon monoxide and, if nickel matte or other impure source of nickel has been treated, impurities. If the nickel carbonyl is to be separated instead of being immediately decomposed in the way usual in the manufacture of nickel, it is liquefied under pressure or otherwise. Liquefaction may be desired either to lead to liquid nickel carbonyl as the final product or, in the case of nickel carbonyl produced direct from mattes or the like, to purify the nickel carbonyl before decomposing it to yield pure nickel. The principal object of the present invention is so to conduct the liquefaction or condensation that the maximum quantity of pure nickel carbonyl is obtained in liquid form.

25 The present invention is based on the remarkable discovery that the saturated vapour pressure of nickel carbonyl is profoundly affected by the partial pressure of carbon monoxide in contact with it. Thus it is found that the vapour pressure decreases until the partial pressure of carbon monoxide reaches a certain critical value, but that when the partial pressure increases above this value the vapour pressure of the nickel carbonyl again increases.

30 According to the present invention this discovery is applied to bring about the liquefaction of the nickel carbonyl under conditions such that its vapour pressure in the condensation space at the condensation temperature is in the neighbourhood of a minimum so that the quantity of liquid nickel carbonyl obtained is at or approaches its maximum for the temperature in question. It is found that the variations in vapour pressure of the nickel carbonyl are conditioned solely by 35 the presence of carbon monoxide, the presence of inert gases or vapours having little or no influence on it. Preferably the conditions are such that the vapour pressure of the nickel carbonyl is not greater than 50 grams of nickel per cubic 40 metre of gas at N.T.P. above the said minimum.

45 In general the invention involves alteration of the pressure from that at which the nickel carbonyl was formed to another pressure, so as to increase the yield of liquid nickel carbonyl. This 50 adjustment may necessitate either raising or

lowering of the pressure in accordance with the pressure at which the nickel carbonyl is formed and the temperature of condensation, and the separation of the liquid from the gaseous phase is effected at the selected higher or lower pressure. 5 Thus the invention is essentially distinguished from processes in which nickel carbonyl formed under pressure is cooled at that pressure and subsequently reduced to atmospheric pressure in stages, since although it will then pass through the optimum pressure, i. e., that at which the maximum yield is obtained, separation is not effected at that optimum pressure. In some cases no adjustment of the pressure is necessary, since the nickel carbonyl may be formed at the optimum 10 condensation pressure and then condensation and separation may take place at that pressure.

15 The relation between the partial pressure of carbon monoxide and the saturated vapour pressure of nickel carbonyl is shown in the accompanying drawing, which represents a graph of isotherms. The partial pressure of carbon monoxide while liquefaction is taking place is plotted isothermally against the nickel content of the 20 gaseous or vapour phase in the liquefaction vessel, reckoned as grams of nickel per cubic metre of gas at N.T.P. Since the gaseous phase may be assumed to be saturated with nickel carbonyl vapour at the temperature under consideration, the ordinates of the curves give a direct measure 25 of the vapour pressure of nickel carbonyl at the condensation temperature. It will be appreciated that the parts of the curves shown in the drawing represent only a small part of the complete 30 curves between 0 and 300 atmospheres and that at very low pressures the vapour pressure of the nickel carbonyl is several times the minimum shown for the temperature in question. The 35 isotherms show a very well defined minimum of nickel carbonyl vapour pressure with respect to 40 carbon monoxide partial pressure and according to the present invention the condensation of the nickel carbonyl is effected in the neighbourhood of this minimum at the particular condensation 45 temperature. Naturally to obtain the best results the pressure is maintained as near to the minimum as possible, but it will be seen that, particularly at the lower temperatures, it is possible to depart fairly substantially from the minimum and still to obtain yields that are relatively 50 high and are far higher than those obtained at atmospheric pressure. It will be noted in particular that between the temperatures of 0 to 40° C. the range of from 10 to 150 atmospheres gives 55 good results. Naturally it is often most conven-

ient to effect the condensation at about atmospheric temperature, but in practice various factors have to be considered and when all these are taken into account the most convenient temperature of condensation may not be found to be atmospheric temperature, nor yet a lower temperature at which an increased proportion of nickel carbonyl could be liquefied. Accordingly a feature of the invention may be stated to consist in effecting the condensation at a carbon monoxide partial pressure between 45 atmospheres less and 75 atmospheres more than that corresponding to the minimum for the condensation temperature selected, which minimum may be ascertained experimentally or determined with the aid of the accompanying drawing. Instead of using the drawing graphically, a convenient manner for determining the carbon monoxide partial pressure at which maximum condensation of nickel carbonyl takes place is to utilize an equation derived from the graphs in the drawing. Thus, the following empirical equation gives the lower limits of the range of carbon monoxide partial pressures at which maximum condensation of nickel carbonyl occurs:  $P=0.6T+22$  in which:

T=the chosen condensation temperature (°C.),

P=the carbon monoxide partial pressure,

22=a constant.

30

This equation is derived from the graphs in the accompanying drawing which depicts a family of isotherms, as those skilled will readily understand. It will be observed that for maximum yield of liquid nickel carbonyl, the condensation takes place within the pressure range of 130 atmospheres carbon monoxide partial pressure and 0.6T+22 atmospheres carbon monoxide partial pressure. Of course the total pressure at which maximum condensation occurs may be calculated, as those skilled in the art know, from the carbon monoxide content of the gases to be condensed and the aforesaid carbon monoxide partial pressure. The preferred limits within which the maximum yield of nickel carbonyl is obtained are indicated in the drawing by the area limited by lines AB and CD and the portions of isotherms segregated by the aforesaid lines AB and CD.

In order to show the advantage obtained by effecting the condensation in the neighbourhood of that carbon monoxide partial pressure which gives the minimum nickel carbonyl vapour pressure, figures obtained with a certain gas mixture will now be given. Carbon monoxide gas containing nickel carbonyl equivalent to 500 gms. of nickel per cubic meter was progressively compressed at 20° C. and the liquid carbonyl thereby condensed is shown in the following table:

| 60 | CO pressure ats. | Percent Ni (CO)<br>liquefied |
|----|------------------|------------------------------|
| 10 |                  | 75.6                         |
| 25 |                  | 87.0                         |
| 50 |                  | 91.2                         |
| 65 | 100              | 90.8                         |
|    | 200              | 82.4                         |
|    | 300              | 61.4                         |

It is clear from this table that the maximum condensation is obtained when the carbon monoxide partial pressure is between 50 and 100 atmospheres, and this fact is of course also shown by reference to the accompanying drawing. Further it will be noticed that the yield at 25 atmospheres is distinctly greater than that at 200 atmospheres.

In carrying the invention into effect either a batch process or a continuous process may be used, the invention being in no way dependent on this. The carbonyl may be formed at lower pressures and then compressed so that the carbon monoxide partial pressure brings the vapour pressure of the nickel carbonyl to the value desired or else the reaction may be conducted at higher pressures followed by expansion to the desired pressure. Alternatively the concentration of carbon monoxide may be varied in order to secure the partial pressure desired.

In order that the invention may be more readily understood two examples of its application will now be given.

15

#### Example I

The exit gases of an atmospheric pressure nickel extraction plant, that is to say, a volatiliser used in the well known Mond carbonyl process, 20 contained nickel carbonyl vapour equivalent to 420 grams of nickel per cubic metre. In order to obtain the maximum yield of nickel carbonyl, these gases were compressed at 0° C. to the optimum carbon monoxide pressure of 55 atmospheres and separation was then effected. The liquid nickel carbonyl obtained in this way was 25 95.4% of that in the gases.

#### Example II

30

Carbon monoxide gases from a high pressure reaction vessel containing nickel carbonyl vapour in an amount equivalent to 450 grams of nickel per cubic metre at a pressure of 250 atmospheres and at 80° C. were expanded to a pressure of 70 35 atmospheres into a "let-down" vessel at atmospheric temperature. Separation was effected at the pressure of 70 atmospheres and the amount of liquid nickel carbonyl obtained was 94% of 40 that in the gases.

We claim:

1. The improved process for liquefying nickel carbonyl which comprises reducing the pressure of gases containing carbon monoxide and about 450 grams of nickel per cubic metre as condensable nickel carbonyl at a reaction pressure of about 250 atmospheres total pressure and a reaction temperature of about 80° C. to a condensation pressure equivalent to a carbon monoxide partial pressure of about 70 atmospheres at a condensation temperature of about normal atmospheric temperature while maintaining said condensation temperature practically constant, liquefying said nickel carbonyl at said carbon monoxide partial pressure, and separating said liquefied nickel carbonyl at said carbon monoxide partial pressure whereby about 94% of 50 said condensable nickel carbonyl is recovered.

2. The improvement in the method for liquefying nickel carbonyl which comprises compressing gases from an atmospheric pressure nickel extractor containing carbon monoxide and condensable nickel carbonyl equivalent to about 420 grams of nickel per cubic metre at normal temperature and pressure in accordance with the carbon monoxide content of said gases to an altered total pressure equivalent to a carbon monoxide partial pressure of about 55 atmospheres at a substantially constant condensation temperature of about 0° C. to liquefy practically all 60 of said condensable nickel carbonyl at said altered pressure, and separating said liquid nickel carbonyl at said carbon monoxide partial pressure.

3. The improved process for the production of nickel carbonyl which comprises reacting nickel- 75

containing material and carbon-monoxide containing gases at a reaction temperature and under a reaction pressure to obtain reaction gases containing carbon monoxide and condensable nickel carbonyl, cooling said gases containing condensable nickel carbonyl from said reaction temperature to a condensation temperature of about 0° C. to about 80° C., altering the total pressure of said cooled gases from said reaction pressure to a condensation total pressure dependent upon the carbon monoxide content of said cooled gases and corresponding to a carbon monoxide partial pressure between about 130 atmospheres and a carbon monoxide partial pressure calculated from the equation,  $P=0.6T+22$ , while maintaining said condensation temperature practically constant, liquefying at least 90% of said condensable nickel carbonyl at said altered pressure, and separating said liquefied nickel carbonyl whilst maintaining said altered condensation pressure substantially constant whereby increased amounts of nickel carbonyl are recovered.

4. A process for obtaining substantially complete condensation of nickel carbonyl in the liquid phase from a mixture of gases including carbon monoxide and nickel carbonyl which comprises establishing a body of said gases at a condensation temperature between about 0° C. and about 80° C. and at a reaction pressure, altering said reaction pressure whilst maintaining said con-

densations temperature practically constant to a condensation total pressure dependent upon the carbon monoxide content of said body of gases and corresponding to a carbon monoxide partial pressure of about 22 to about 130 atmospheres, liquefying at least 90% of said condensable nickel carbonyl present at said altered pressure, and separating liquid nickel carbonyl from the overlying gas and residual vapor mixture whilst maintaining and altered pressure practically constant. 5 10

5. A process for obtaining substantially complete condensation of nickel carbonyl in the liquid phase from a mixture of gases containing nickel carbonyl and carbon monoxide under a total pressure in excess of 100 atmospheres which comprises reducing the total pressure on said mixture of gases to an altered total pressure dependent upon the carbon monoxide content of said mixture and corresponding to a carbon monoxide partial pressure between about 130 atmospheres and a carbon monoxide partial pressure dependent upon a condensation temperature not greater than about 100° C. and calculated from the equation,  $P=0.6T+22$ , liquefying nickel carbonyl whilst maintaining said pressure practically 15 20 25 constant, and separating said liquefied nickel carbonyl whilst maintaining said altered pressure substantially constant.

CHARLES F. R. HARRISON. 30  
ALBERT EDWARD WALLIS.